# EUROPEAN PATENT SPECIFICATION

(11) **EP 0 843 750 B1**
(45) Date of publication and mention of the grant of the patent: **10.05.2000**
(21) Application number: 95929383.8
(22) Date of filing: 04.08.1995
(51) Int. Cl.: D01F 6/62, D01D 5/08, D02J 1/22

(54) **MAKING HIGH FILAMENT COUNT FINE FILAMENT POLYESTER YARNS**
VERFAHREN ZUR HERSTELLUNG VON POLYESTERGARNE MIT EINER HOHEN ANZAHL VON FEINFILAMENTEN
FABRICATION DE FILS DE FILAMENT DE POLYESTER, DE TITRE FIN, A NOMBRE DE FILAMENTS ELEVE

(43) Date of publication of application: 27.05.1998
(73) Proprietor: E.I. DU PONT DE NEMOURS AND COMPANY, Wilmington Delaware 19898 (US)
(72) Inventor: BENNIE, David, George, Rocky Point, NC 28457-9560 (US); COLLINS, Robert, James, Wilmington, NC 28405-9366 (US); FRANKFORT, Hans, Rudolf, Edward, Winterville, North Carolina 28590 (US); JOHNSON, Stephen, Buckner, Wilmington, NC 28409 (US); KNOX, Benjamin, Hughes, Wilmington, DE 19808-5420 (US); LONDON, Joe, Forrest, Jr., Greenville, NC 27858-5621 (US); MOST, Elmer, Edwin, Jr., Durham, NC 27707-5276 (US); PAI, Girish, Anant, Matthews, NC 28105-8843 (US)
(74) Representative: Jones, Alan John
(86) International application number: US9509909
(87) International publication number: WO9706295

(56) References cited:
- WO-A-92/13119
- WO-A-94/03661
- DATABASE WPI Section Ch, Week 9317 Derwent Publications Ltd., London, GB; Class A23, AN 93-140727 XP002002106 & JP,A,05 078 911 (NIPPON ESTER CO LTD) , 30 March 1993
- DATABASE WPI Section Ch, Week 7934 Derwent Publications Ltd., London, GB; Class A23, AN 79-62363B XP002002107 & JP,A,54 088 316 (TORAY INDS INC) , 13 July 1979
- DATABASE WPI Section Ch, Week 9347 Derwent Publications Ltd., London, GB; Class A23, AN 93-375520 XP002002108 & KR,B,9 303 356 (KOLON CO) , 26 April 1993
- PATENT ABSTRACTS OF JAPAN vol. 012, no. 122 (C-488), 15 April 1988 & JP,A,62 243824 (TEIJIN LTD), 24 October 1987,

## Description

The invention concerns improvements in and relating to melt-spinning fine continuous filament polyester yarns and particularly to an improved process for preparing such yarns of high filament count (HFC) having improved uniformity such as makes these yarns especially suitable for textile end-uses that may require downstream processing without breaking filaments and for use in dye-critical textile applications.

Polyester filament yarns of denier per filament (dpf) less than about 1 (i.e., similar to the dpf of silk), are commercially available, but are more costly to make than filament yarns of more conventional dpf (similar to that of cotton). Our so-called "parent" application No. 07/647,371 (now abandoned in favor of a continuation-in-part application now issued as U.S. Patent No. 5,250,245, as was a companion case, now issued as U.S. Patent No. 5,288,553, the disclosure of both of which are hereby incorporated herein by reference) was concerned with the preparation of such fine filaments by a novel direct melt-spinning process. Reference is also made to related WO-A-92 13119.

Reaction in the trade to the fine filament textile (flat or textured) yarns has tended to limit their use in textile fabrics unless the total yarn denier (D_{Y}) of the fine filament yarn is approximately the same as that of the higher dpf yarn that it replaces. For example, if an incumbent yarn has filaments of denier 1.5 dpf (and we shall refer to this incumbent yarn as a low filament count (LFC) yarn) is to be replaced by a finer filament yarn whose filaments are of half the dpf of the LFC yarn, i.e., 0.75 dpf, then the number of filaments in the finer filament (0.75 dpf) yarn needs to be approximately twice that of the incumbent LFC yarn to be a direct replacement in existing textile end-uses, i.e., to provide the same fabric weight (grams/meters²). In other words, an LFC yarn of, for instance, 100 filaments and 150 denier (i.e., 1.5 dpf), should be replaced by an HFC yarn, also of 150 denier, but of 200 filaments, on account of the lower 0.75 dpf. Some fiber producers have, therefore, spun two (or more) separate smaller fine filament "bundles" and have then co-mingled (interlaced) the separate smaller bundles to provide a single HFC yarn of the desired total yarn denier (D_{Y}) equal to that of the larger dpf LFC yarn that is to be replaced. They have done this despite the loss in spinning productivity this separate spinning has entailed; the loss in spinning productivity results from the fact that two (or more) spinnerets are used to provide filaments for only one yarn. The reason for using more spinnerets has been a belief, based on previous experience with spinning filaments of higher dpf, that, to maintain satisfactory quality levels (along-end denier, structure uniformity and mechanical quality are the criteria used by us), it has not been desirable to increase the number (#) of filaments spun per "useful" extrusion area in the face of the spinneret (referred to herein as filament extrusion density (FED), given as #/cm²) significantly over what was previously used to spin the larger dpf LFC yarn. If a customer were to receive from a fiber producer separate smaller fine filament yarns of low yarn denier, the customer would want to co-mingle two or more of these smaller fine filament yarns to obtain the desired total yarn denier (D_{Y}), which would be an added cost to him in making the final textile yarn. Also co-mingling filament yarns that have been spun separately has not provided the same visual fabric aesthetics (or dye uniformity) as provided by interlacing a single HFC bundle of the same yarn denier (D_{Y}). In other words, there has been a significant detectable difference in aesthetics and/or performance between a plied yarn and a unitary interlaced yarn.

Accordingly, it has been desirable to provide a melt-spinning process for spinning a single HFC bundle of fine dpf filaments from a single extrusion spinneret (i.e., without the need for plying two or more filament bundles) and thereby not sacrificing spinning productivity, while maintaining required along-end uniformity and mechanical quality for down-stream processing of the HFC fine filament yarn.

According to the invention, there is provided a process of preparing by melt-spinning an interlaced multifilament (HFC) yarn of at least 150 fine filaments in number (#) and of 0.5 to 2.2 spun denier per filament (dpf)ₛ, from a polyester polymer of 13 to 23 relative viscosity (LRV) and of 240°C to 265°C zero-shear melting point (Tₘ^{o}) comprising :-
(i) melting the polyester polymer, heating the resulting melt to a polymer temperature (Tp) that is 25°C to 55°C above the Tₘ^{o}, and filtering the heated melt;
(ii) extruding the filtered melt through at least 150 capillaries in the face of a spinneret to form the aforesaid number (#) of at least 150 filamentary streams at a filamentary extrusion density (FED) of at least 6 filaments/cm² and at a total melt mass flow rate W, in g/min, the total melt mass flow rate of all these streams being W (= w x #) where w is the mass flow rate through a single capillary and ${\text{= (dpf)}}_{\text{s}} {\text{x (V}}_{\text{s}} \text{)/9000}$, where Vₛ is the spinning withdrawal speed and is at least 2Km/min;
(iii) protecting the freshly-extruded filamentary streams immediately below the face of the spinneret by a delay shroud (of length L_{q} cm below said face), then cooling them by quenching air of laminar velocity (Qₐ m/min), such that the Spin Factor SF is 0.2 to 1, where said Spin Factor (SF) is calculated according to the expression:${\text{SF = k{(LRV)[T}}_{\text{m}} {}^{\text{o}} {\text{+25)/(Tp)]}}^{\text{6}} {\text{[(V}}_{\text{s}} {\text{)}}^{\text{2}} {\text{/(dpf)}}_{\text{s}} {\text{][(Q}}_{\text{a}} {\text{/W)}}^{\text{0.2}} {\text{][(FED) (L}}_{\text{q}} {\text{)}}^{\text{-0.7]}} {\text{}}}^{\text{n}}$ where "k" = 2.4x10⁺⁵ and 'n' = minus (-) 0.8;
(iv) cooling the filamentary streams to a temperature below T_{g}, converging the resulting cooled filaments into a single multifilament bundle of at least 150 filaments at a convergence distance (L_{c}, in cm) from the face of the spinneret, and interlacing the single multifilament bundle to provide an interlaced spin-oriented yarn;
   and wherein the interlaced yarn is wound to form a package at a winding speed of 2 to 5 Km/min.

As indicated, the Spin Factor (SF) is important; it is defined by the expression:${\text{SF = k[η}}_{\text{a}} {\text{σ}}_{\text{F}} {\text{Q}}_{\text{F}} {\text{]}}^{\text{n}} \text{,}$ and in the "expanded" form by the expression used herein:${\text{SF = k{(LRV)[T}}_{\text{m}} {}^{\text{o}} {\text{+25)/(Tp)]}}^{\text{6}} {\text{[(V}}_{\text{s}} {\text{)}}^{\text{2}} {\text{/(dpf)}}_{\text{s}} {\text{][(Q}}_{\text{a}} {\text{/W)}}^{\text{0.2}} {\text{][(FED) (L}}_{\text{q}} {\text{)]}}^{\text{-0.7}} {\text{]}}}^{\text{n}}$ where$\begin{matrix}\begin{matrix}{\text{k = 2.4x10}}^{\text{5}} \\ \text{n=minus (-) 0.8} \\ {\text{ηa (apparent melt viscosity)=(LRV)[T}}_{\text{m}} {}^{\text{o}} {\text{+25)/(T}}_{\text{P}} {\text{)]}}^{\text{6}} \\ {\text{σF(spinline stress factor)=(V}}_{\text{s}} {\text{)}}^{\text{2}} {\text{/(dpf)}}_{\text{s}} \\ {\text{QF (quench factor)=[(Q}}_{\text{a}} {\text{/W)}}^{\text{+0.2}} {\text{][(FED)(L}}_{\text{q}} {\text{)}}^{\text{-0.7}} \text{]} \\ \text{W(g/min/extrusion bundle)=(# filaments)x(w)} \\ {\text{w (g/min/capillary)=[(dpf)}}_{\text{s}} {\text{x V}}_{\text{s}} \text{(m/min)/9000]} \\ {\text{Q}}_{\text{a}} \text{=laminar air flow in meters per minute} \\ {\text{FED = # filaments per "useful" extrusion area in cm}}^{\text{2}} \\ {\text{L}}_{\text{q}} \text{=delay quench length in cm;}\end{matrix}\end{matrix}$ and where all three of ηₐ, σ_{F}, and Q_{F} should be balanced as indicated in the above relationship to give a Spin Factor (SF) of 0.2 to 1 in order to spin uniform fine filament (HFC) yarns according to the invention.

The document WO9213119 discloses already an empirical relationsship in order to control the spinning of polyester yarns, grouping the stress factors, the result being an internal spinning stress σa. It has been found, that the quench parameters could also been introduced into this formula, giving a characterising spin factor, useful to control the spinning.

Quality levels of the filaments are desirably measured by along-end denier (i.e., a low Denier Spread (DS), desirably less than 2.5%, particularly less than about 2.0%, preferably less than about 1.5%, and especially about 1.0% or less, it being understood that these uniformity criteria are increasingly difficult to obtain as the dpf is reduced), structure uniformity (as measured by the along-end draw tension (coefficient of) variation (DTV,%) which should desirably be less than 1%, and is discussed more in detail in relation to Spin Factor (SF), especially referring to Figure 1, hereinafter) and mechanical quality (as measured by normalized tenacity-at-break-denier (T_{B})ₙ, where ${\text{(T}}_{\text{B}} {\text{)}}_{\text{n}} {\text{= Tenacity (g/d)(RDR)}}_{\text{s}} {\text{(20.8/LRV)}}^{\text{0.75}}$, as discussed later, where (RDR)ₛ is the residual spun draw ratio and is defined by ${\text{(RDR)}}_{\text{s}} {\text{= [1 +(E}}_{\text{B}} \text{)/100]}$, where (E_{B}) is the percentage elongation-to-break).

As will be discussed, capillary dimensions herein and in the art (D for diameter and L for length) can be extremely important. Such dimensions are preferably such that the L/D ratio is at least 2, and the L/D⁴ value is at least 335 mm⁻³.

By this new melt-spinning process, according to the present invention, it has been possible to achieve a melt-spinning productivity of at least 5000, where melt-spinning productivity (Pₛ) is given as the product of the withdrawal speed (Vₛ) in m/min and the residual spun draw ratio (RDR)ₛ of the spin-oriented filaments according to the expression, (${\text{P}}_{\text{s}} {\text{=V}}_{\text{s}} {\text{x(RDR)}}_{\text{s}}$), and (RDR)ₛ is given by ${\text{(RDR)}}_{\text{s}} {\text{=[1 +(E}}_{\text{B}} \text{)/100]}$, where (E_{B}) is the percentage elongation-to-break.

The resulting interlaced multi-filament yarns are believed new, as will be indicated, because they number at least 150 filaments of fine denier, up to 2.2 spun dpf (dpf)ₛ, and up to 1 dpf, when drawn, and yet their filament entanglement shows unitary interlace. They show desirable uniformity, as expressed for the filaments by low DTV values, and desirably by low DS, and for the yarns by high (T_{B})ₙ values, as indicated.

Some of the spin-oriented yarns may be used as such, i.e., in as-spun condition as "direct-use" yarns, and most of them may be drawn in a coupled or split process, single-end or in a form of a sheet of few ends, or in the form of a weftless warp sheet, to provide drawn flat multi-filament yarns having a residual elongation as desired, generally between about 15% to about 40%, and normalized (T_{B})n values of at least 5 g/dd, preferably of at least 5.5 g/dd, and especially of at least 6 g/dd. Such drawing may be incorporated as part of a split or coupled draw-texturing process, such as draw air-jet texturing or draw false-twist texturing, in which case the yarns may be drawn to somewhat higher elongation, e.g. up to about 45%. The yarns may, if desired, be subjected to a compression crimping process (e.g., stuffer-box crimping).

The HFC yarns of the invention (whether spun or drawn, flat or textured yarns) have unitary interlace and have at least 150 filaments, preferably at least 175 filaments and especially at least 200 filaments. As indicated, the spun denier (dpf)ₛ of the as-spun filaments is desirably 0.5 to 2.2, and preferably 0.6, 0.65 or 0.7 on up, e.g., to about 2 (dpf)ₛ. The denier per filament of the drawn (e.g., flat or draw-textured) HFC yarns of the invention desirably have a filament denier of about 1 or less and generally up to about 0.8, e.g. 0.2 to 0.8 dpf. Draw-textured HFC yarns of the invention are further characterized by an elongation-to-break of 15% to 45%, a normalized tenacity-at-break-denier of at least 4 g/dd, preferably at least 4.5 g/dd, and a Toray Fray Count of less than 10 per 1000 meters, preferably less than 5 per 1000 meters. Indeed, as may be seen in the Examples, Fray Counts of 0 have been achieved according to the invention.

High filament count (HFC) post-bulkable yarns may be prepared by spinning and gently heat-setting an HFC mixed-filament yarn comprised of two or more types of filaments that differ in denier and/or cross-section under conditions selected such as to provide a potential differential shrinkage (because of differential crystallinity) between the filament types, i.e. sufficient to preserve a shrinkage difference of at least 5% (i.e., not to over heat set), and such that when the drawn mixed-filament yarn is heated under relaxed conditions the differing filaments of the HFC drawn mixed-filament yarn still have sufficient differential shrinkage to shrink differentially and so give a yarn having different filament lengths (giving along-end loops) and thereby provide an HFC bulky yarn comprised of core filaments (previously of high shrinkage) having a (dpf)_{core} greater than the dpf of the surface filaments (previously of lower shrinkage). In HFC mixed-shrinkage yarns of the invention the surface filaments after boil-off shrinkage (ABO) desirably have a (dpf)_{ABO} of less than 1, and preferably less than 0.8; and the total yarn average (dpf)_{Y} (after boil-off) should generally be less than 1 (as shown, e.g., in Example 5).

Further aspects and embodiments of the invention will appear hereinafter.
Figure 1 is a plot of draw tension variation (DTV,%) versus the Spin Factor SF, defined hereinbefore. Undrawn yarns of the invention preferably have DTV-values of less than 1%, and are spun so the SF is in the range of 0.2 to 1 as shown by the lightly dashed lines. Preferred combinations of DTV and SF-values for making preferred yarns of the invention are represented by the shaded area/////// between Lines A and C, where Lines A and C have the formula $\text{DTV = a(SF) +b}$, wherein a = 1 and b = +0.2 and -0.2 for Lines A and C, respectively (on either side of especially preferred Line B, expressed similarly, except that b=0 for line B), and where the DTV and SF values are both between 0.2 and 1.
Figure 2 is a representative plot of percent boil-off shrinkage (S) versus percent elongation-to-break (E_{B}) wherein straight Lines 1, 2, 3, 4, 5, 6, 7, and 8 represent (1-S/Sₘ)-values of 0.85, 0.7, 0.6, 0.4, 0.2, 0.1, 0.05, and 0, respectively, and curved Line 9 represents a typical shrinkage versus elongation-to-break relationship for a series of yarns formed, for example, by increasing spinning speed, but keeping all other process variables unchanged. Changing other process variables (such as dpf, polymer viscosity) produces a "family" of similar curved lines that are of essentially similar configurations. The vertical dashed lines denote ranges of E_{B}-values for preferred filaments of the invention, i.e., E_{B} values of 40% to 175%, with 160% as a practical upper limit, based on age stability, and especially up to 140%.
   Preferred filaments of the invention denoted by the "widely-spaced" //////-area are especially suitable as draw-feed yarns, being defined by E_{B}-values of about 90% to 160% and (1-S/Sₘ) value of at least about 0.05 (line 7).
   Preferred filaments of the invention especially suitable for direct-use, i.e. without further drawing and/or heating, are denoted by the "densely-spaced" \\\\\\-area bordered by E_{B}-values of about 40% to about 90% and (1-S/Sₘ) ratio at least about 0.85 (line 1).
   The expression (1-S/Sₘ) is used herein as a relative degree of stress-induced crystallization (SIC). Sₘ is the expected maximum shrinkage potential for filaments of a given degree of molecular extension (E_{B}) in the absence of crystallinity, and may be calculated as follows:-${\text{S}}_{\text{m}} {\text{(%) = ([E}}_{\text{B}} {\text{)}}_{\text{max}} {\text{-E}}_{\text{B}} {\text{)]/[(E}}_{\text{B}} \text{)max+100])100%,}$ wherein (E_{B})ₘₐₓ is the expected maximum elongation-to-break (E_{B}) of totally amorphous "isotropic" filaments. For polyester filaments spun from polymer of typical textile viscosities LRV-values of about 13 to about 23), the nominal value of (E_{B})ₘₐₓ is experimentally found to be about 550% providing for a maximum residual draw-ratio of 6.5 (Reference: High-Speed Fiber Spinning, ed. A. Ziabicki and H. Kawai, Wiley-Interscience (1985), page 409) and thus, Sₘ (%) is defined, herein, by the simplified expression:${\text{[(550-E}}_{\text{B}} \text{)/650] x100%}$
Figures 3 and 4 are partial schematic representations of partial spinneret arrangements having high filament extrusion density (FED). The arrays are designed to optimize flow of cooling air through the extrusion bundle, and to minimize coalescence of freshly-extruded filaments and poor spinning performance and poor along-end uniformity of the quenched filament bundle. Such arrangement is described in allowed application No. 08/214,717 (DP-4555H), filed by Aneja et al. on March 16, 1994, from which the 5-ring arrangement of Fig. 3 was taken, merely for convenience. The orifices can be arranged in more rings to give an HFC yarn, while being staggered similarly, so as to increase the number of filaments spun from a single spinneret. This is shown in Fig. 4 for spinning 200 filaments from a single spinneret.

The polyester polymer used for preparing spin-oriented filament yarns of the invention is the same as for the "parent" application; that is, the polyester polymer is an ethylene terephthalate polymer selected to have a relative viscosity (LRV) in the range about 13 to about 23, a zero-shear melting point (Tₘ^{o}) in the range about 240°C to about 265°C; and desirably a glass-transition temperature (T_{g}) in the range about 40°C to about 80°C (wherein Tₘ^{o} and T_{g} are measured from the second DSC heating cycle under nitrogen gas at a heating rate of 20°C per minute). The said polyester polymer is a linear condensation polymer composed of alternating A and B structural units, where the A's are hydrocarbylene dioxy units of formula [-O-R'-O-] and the B's are hydrocarbylenedicarbonyl units of formula [-C(O)-R''-C(O)-], wherein R' is primarily [-C₂H₄-], as in the ethylenedioxy (glycol) unit [-O-C₂H₄-O-], and R'' is primarily [-C₆H₄-], as in the 1,4-phenylenedicarbonyl unit [-C(O)-C₆H₄-C(O)-], such as to provide sufficient ethylene terephthalate [-O-C₂H₄-O-C(O)-C₆H₄-C(O)-] repeat groups so as to maintain the Tₘ^{o} between about 240°C and about 280°C. Suitable poly(ethylene terephthalate)-based polymer (herein denoted as PET or 2GT) may be formed by a DMT-process, e.g., as described by H. Ludewig in his book "Polyester Fibers, Chemistry and Technology", John Wiley and Sons Limited (1971), or by a TPA-process, e.g., as described in Edging U. S. Patent No. 4,110,316. Included are also copolyesters in which, for example, up to about 15 percent (or even 20 percent) of the hydrocarbylenedioxy and/or hydrocarbylenedicarbonyl units are replaced with different hydrocarbylenedioxy and hydrocarbylenedicarbonyl units to provide enhanced low temperature disperse dyeability, comfort, and aesthetic properties. Suitable replacement units are disclosed, e.g., in Most U. S. Patent No. 4,444,710 (Example VI), Pacofsky U. S. Patent No. 3,748,844 (Col. 4), and Hancock, et al. U. S. Patent No. 4,639,347 (Col. 3).

Polyester polymers, used herein, may, if desired, be modified by incorporating ionic dye sites, such as ethylene-5-M-sulfo-isophthalate residues, where M is an alkali metal cation, for example in the range of about 1 to about 3 mole percent. To adjust the dyeability or other properties of the spin-oriented filaments and the drawn filaments therefrom, some diethylene glycol (DEG) may be added to the polyester polymer as disclosed by Bosley and Duncan U. S. Patent No. 4,025,592 and in combination with chain-branching agents as described in Goodley and Taylor U. S. Patent No. 4,945,151. To enhance dyeability with disperse dyes, copolyesters may be used as mentioned in Most U. S. Patent 4,444,710, Pacofsky U. S. Patent 3,748,844, Hancock U. S. Patent 4,639,347, and Frankfort and Knox U. S. Patents 4,134,882 and 4,195,051. To overcome the higher shrinkage of copolyester yarns (if considered undesireable for a given end-use), representative branching agents may be used to reduce shrinkage as mentioned in Knox U. S. Patent 4,156,071 , MacLean U. S. Patent 4,092,229, and Reese U. S. Patents 4,883,032, 4,996,740, and 5,034,174; and polymer of higher viscosity (e.g., by about +0.5 to about +1.0 LRV units) may be used to control yarn shrinkage (e.g., the extent of crystallization).

Most of the details of the melt-spinning process have been described in U.S. Patents Nos 5,250,245 and 5,288,553, so need not be repeated. The polymer is heated to a temperature (T_{P}) and extruded through capillaries of preferred dimensions, as indicated, such that L/D⁴ is at least 335 mm⁻³, and the freshly-extruded filamentary streams are immediately protected by a short delay shroud (preferably of length 2 to 5cm), and then quenched, preferably radially, as described by Dauchert in U.S. Patent No. 3,067,458 and Examples 1, 2 and 11 of Knox U.S. Patent No. 4,156,071, to form solid filaments that are preferably converged into a single bundle by metered finish tip applicator guides, as described, e.g., by Agers in U.S. Patent No. 4,926,661, selecting the convergence length (L_{c}) to balance the desire for low downstream air drag (giving high winding tensions) vs. desire for optimum quenching air flow (to provide low DTV and low DS). Typically the withdrawal speed is controlled by use of a feed roll, which preferably cooperates with a let down roll before the windup, using an S-wrap configuration. The single filament bundle is intelaced to provide a unitary interlaced yarn, as described by Bunting and Nelson in U.S. Patent No. 2,985,995 and by Agers in U.S. Patent No. 4,926,661. The interlace is conveniently measured by conventional means, e.g., as in Hitt U.S. patent No. 3,290,932 or wit a Rothschild device to give a pin count, which is an average of several readings.

Generally, untextured filaments and yarns are referred to herein as "flat", and as-spun (undrawn) flat yarns intended for drawing as "feed" or as "draw-feed" yarns. As-spun (undrawn) yarns which can be used as a "textile" yarn without need for further drawing and/or heat treatment are referred to herein as "direct-use" yarns. For textile purposes, a "textile" yarn should generally have certain minimum properties, such as sufficiently high modulus and yield point, and sufficiently low shrinkage, which distinguish such "textile" yarns from conventional feed yarns that require further processing before they have the minimum properties for processing into textiles and subsequent use. It will be recognized that, where appropriate, our technology teaching may apply also to polyester filaments in other forms, such as bundles or tows, which may then be converted into staple fiber, and used as such in accordance with the balance of properties that is desirable and may be achieved as taught hereinafter.

As indicated, a main purpose of the present invention has been to solve the productivity problems and disadvantages of the prior art, namely having to melt spin separate filament bundles of lower number of filaments and having to combine 2 or more such separate filament bundles to provide the desired total yarn denier (D_{Y}) by interlacing or co-mingling such lesser bundles (having less filaments) to provide the desired total yarn denier (D_{Y}) prior to draw-warping or after draw-texturing and, in doing this, to provide filaments of sufficient along-end structural uniformity, measured herein by along-end draw tension variation (DTV,%), along-end denier spread (DS,%), which indicates sufficient physical uniformity, and mechanical quality, as measured by the yarn tenacity-at-break-denier normalized to a polymer LRV of 20.8, for use in textile processing (i.e., providing uniform textile yarns with essentially no broken filaments, herein referred to as "frays"). As indicated, we have achieved this by careful selection of polymer (LRV and Tₘ^{o}) and process conditions to provide a spin factor (SF) in the range of 0.2 to 1, and especially such that DTV,% is less than 1, e.g. 0.2 to 1, and also between [SF + 0.2] and [SF - 0.2]; In other words, as indicated hereinbefore, these factors are important, according to the invention:- η_{a,} referred to as the "apparent" melt viscosity at temperature T_{P}; σ_{F} the spinline stress factor; and Q_{F} the quench factor; all three of these should be balanced as indicated, to spin uniform fine dpf HFC yarns from a single spinneret according to the invention.

Fine filament yarns of this invention may be subjected to warp drawing, air-jet texturing, false-twist texturing, gear crimping, and stuffer-box crimping, for example.

Generally, when draw-texturing fine dpf feed yarns on false-twist texturing (FTT) machines that are characterized by a "bent double heater configuration" (such as a Barmag FK900, and herein denoted as Process A), very high Toray Fray Counts (broken filaments) of 500 to 1000 per 1000 meters have been obtained. When, however, we have inserted a device into the draw-texturing threadline to reduce the twist-induced draw by reducing the break angle between the first upstream contact point and the first friction twist insertion point to less than 15 degrees and to increase the radius of curvature of the upstream contact to greater than 2.5 mm, we have significantly reduced (essentially eliminated) the numbers of broken filaments (frays) when texturing on conventional "bent configuration" FTT machines (as shown in Examples 2 and 3); this technique is denoted herein as Process B (according to our invention). For those who have a Barmag FK900 or other "bent configuration" FTT machine, Process B is far preferable to more expensive solutions, such as modifying the "bent configuration" to eliminate this "twist trap" phenomenon by moving the heater and/or spindle, or replacing the existing "bent" machines and buying "tall" linear configuration FTT machines, or buying Murata belt machines, which are more costly solutions than Process B (one aspect of this invention).

Our new filaments (and bundles/tows made therefrom) may be crimped, if desired, and cut into staple and flock. Fabrics made from these improved yarns may be surface-treated by conventional sanding and brushing to give suede-like tactility. Our new low shrinkage filament yarns may be used as direct-use flat textile yarns. The new yarns may be used as feed yarns for air-jet texturing and stuffer-box crimping, wherein no drawing need be carried out. The improved combination of filament strength and uniformity makes these filaments especially suited for end-use processes that require fine filament yarns without broken filaments (or filament breakage), and/or require uniform dyeing with critical dyes. Fine denier filament polyester yarns of the invention are especially suitable for making high-end density moisture-barrier fabrics, such as rainwear and medical garments. The surface of the knit and woven fabrics can be napped (brushed or sanded). To reduce the denier even further, the filaments may be treated (preferably in fabric form) with conventional alkali procedures.

Our new fine filaments, especially those capable of being cationic dyeable, may also be used as coverings for elastomeric yarns (and strips), preferably by air entanglement as described by Strachan in U. S. Patent No. 3,940,917. The fine filaments of the invention may be co-mingled on-line during spinning or off-line with higher denier polyester (or nylon) filaments to provide for cross-dyed effects and/or mixed-shrinkage post-bulkable potential, where the bulk may be developed off-line, such as overfeeding in presence of heat while beaming/slashing or in fabric form, such as in the dye bath. The degree of interlace and type/amount of finish applied during spinning may generally be selected based on the textile processing needs and final desired yarn/fabric aesthetics. The filament surface frictional characteristics may be changed by selection of cross-section, delusterants, and through such treatments as alkali-etching Further, the frictional characteristics may be enhanced to be more silk-like by use of silicon dioxide versus titanium dioxide delusterants. Other inert metal oxides may be used as delusterants. The spin-oriented polyester filaments, used herein, may advantageously be treated with caustic applied to freshly-extruded filaments, as described by Grindstaff and Reese U.S. Patents Nos. 5,069844, 5069,845 and 5,069,846 to provide the polyester filaments with improved moisture-wicking properties, more akin to those of the nylon filaments.

Indeed, further modifications will be apparent, especially as these and other technologies advance. For example, any type of draw winding machine may be used; post heat treatment of the feed and/or drawn yarns, if desired, may be applied by any type of heating device (such as heated godets, hot air and/or steam jet, passage through a heated tube, microwave heating, etc.); finish application may be applied by convention roll application, herein metered finish tip applicators are preferred and finish may be applied in several steps, for example during spinning prior to drawing and after drawing prior to winding; interlace may be developed by using heated or unheated entanglement air-jets and may be developed in several steps, such as during spinning and during drawing and other devices may be used, such as use of tangle-reeds on a weftless sheet of yarns.

The invention lends itself to further variations and ways to take advantage of the benefits of the yarns of the invention in various drawing and/or heat treatment processes as described hereinafter. As will be understood, feed filaments may be supplied and/or processed according to the invention in the form of a yarn or as a bundle of filaments that does not necessarily have the coherency of a true "yarn", but for convenience herein a plurality of filaments may often be referred to as a yarn or bundle, without intending specific limitation by such term.

### TEST METHODS

Many of the test methods are detailed in the "parent" application and in U.S. Patent Nos. 4,123,882, 4,156,071, 5,066,4475 and in 5,288,553, and are incorporated herein by reference, so further detailed discussion herein would be redundant.

Broken filaments, especially of textured yarns were measured by a commercial Toray Fray Counter (Model DT 104, Toray Industries, Japan) at a linear speed of 700 mpm for 5 minutes i.e., number of frays per 3500 meters, and then the numbers of frays are expressed herein as the number of frays per 1000 meters.

The draw tension variation (DTV) was measured on the DuPont "Draw Tension Instrument"at a draw-ratio of 1.707X for as-spun yarns having elongations of at least 90% at 185°C over a heater length of 1 meter at 185 ypm (169.2 mpm) wherein casablanca type rolls (vs. nip rolls) are used to control tension. For information about the DuPont machine and its availability, questions may be directed to the Engineering R&D Division at E. I. DuPont de Nemours and Company, Wilmington, Delaware 19898. Another instrument brand that uses similar principles (but should be calibrated opposite a DuPont machine) is DYNAFIL, manufactured by TEXTECHNO; this is a fixed-strain device which uses a non-contact heater (length about 30 inches), and normal set up is a 1.6X draw ratio.

The following Examples further illustrate the invention, in showing preparation of multifilament HFC yarns of more than 150 filaments by spinning such filaments in a single bundle from a single spinneret, and subsequent processing of such HFC yarns, and are not intended to be limiting.

### EXAMPLE 1

We have spun a large number of multi-filament HFC yarns from 2G-T polyester polymer of nominal 21.2 LRV and having a zero-shear melting point Tₘ^{o} of 255 C at varying filament extrusion densities (FED). Process and product details of some of these are summarized in Table I. The lowest dpf listed was down to 0.6 dpf (a 150 denier, 250 filament yarn). Such lower dpf as-spun yarns are described hereinafter in Example 4. Comparative items are denoted by the letter C, such as in Item 6C. Yarns having a DTV less than 0.75% are denoted by a letter "P" for preferred. Yarns having denier spread (DS) values in the range of 2 to 2.5% are denoted by the letter "N" (indicating not preferred but according to the invention). Yarns having a preferred normalized tenacity-at-break-denier (T_{B})ₙ of at least 6 g/dd are denoted by a letter "T". Yarns having elongation-to-break (E_{B}) values in the range of 160 to 175% are noted by the letter "E", as such yarns have lower age-stability than draw-feed yarns of lower elongation-to-break, e.g., of 90-160%, (preferably 90-140%). Yarns 1 to 46, 84 to 150, and 159 to 185 were melt-spun using spinneret capillaries of length (L) 36 mil (0.914 mm) and diameter (D) 9 mil (0.229 mm). Yarns 47 to 83 were melt-spun using spinneret capillaries of LxD 21 mil x 7 mil (0.533 mm x 0.178 mm). Yarns 151 to 158 were melt-spun using spinneret capillaries of LxD 18 mil x 6 mil (0.457 mm x0.152 mm). Yarns 1 to 46 were 168 filament yarns spun from a spinneret having a FED of 6.54 #/cm ²; yarns 47 to 150 were 200 filament yarns spun from a spinneret having a FED of 7.7 #/cm²; yarns 151 to 158 were 204 filament yarns spun from a spinneret having a FED of 7.94 #/cm²; and yarns 159 to 185 were 250 filament yarns spun from a spinneret having a FED of 9.74 #/cm².

As indicated (by the Comparative "C" items), we found that the spinning performance of these HFC yarns deteriorated as the FED increased. To overcome this deterioration, our first step was to check and optimize standard process variables and equipment, such as assuring uniform air flow, and optimizing proper convergence length (i.e., long enough to permit convergence without sticky filaments, but short enough to reduce increase in spinline tension from air drag and thereby permit winding up the yarns at lower tensions) and setting the polymer temperature to provide good polymer quality (without thermal degradation). We found this first step improved the spin performance somewhat, but was still sometimes unacceptable. Our next step was to reconsider the extrusion/quenching process. It was unacceptable for us to reduce FED by double-ending (spinning from 2 packs instead from a single pack) since this would cut productivity by 50%. Our objective was to improve yarn mechanical quality (T_{B})ₙ, along-end denier (DS), and along-end structure (DTV) without double-ending. The spin factor (SF) expression defines an approach to the spinning process as an integrated system and permits selection of process variables according to our invention, to achieve desired yarn property goals. The next step would be to "fine-tune" by careful selection of process variables so as to maintain spin performance and yarn uniformity/quality, at a higher spin productivity Pₛ defined by the product of the spin speed (Vₛ) and (RDR)ₛ. Item 14 in Table I is an illustration of the successful use of SF to obtain (T_{B})ₙ greater than 6g/dd, denier spread (DS) no more than 1% and draw tension variation (DTV,%) no more than 0.75%.

We also observed that the capillaries of LxD 21 x 7 mil (0.533 x 0.178 mm) gave an over all better spinning process than the capillaries of LxD 36 x 9 mil (0.914 x 0.229 mm) at the same mass flow rate. Capillaries have previously been characterized by their [L/D⁴] ratio (e.g. in USP. No 4,134,882). In metric units the 6x18 mil, 7x21 mil, and 9x36 mil capillaries have [L/D⁴, mm⁻³] values of 848, 534 and 335, respectively. According to the process of this invention, [L/D⁴] metric values of at least 335 are preferred, and at least 500 is especially preferred.

The filament arrays were optimized for uniform quenching (as described in relation to Figure 3 and in more detail in allowed application No. 08/214,717 (DP-4555-H), referred to above). For calculating the spin factor (SF), those process parameters not included in Table I may be calculated as described hereinbefore. The type and level of spin finish and interlace were selected based on intended end-use; for example, feed yarns for false-twist texturing have lower levels of interlace than those used as feed yarns for draw-warping.

All these yarns are characterized by "random" unitary interlace, i.e., along-end filament entanglement, because all the filaments in each yarn were spun from a single spinneret. Yarns that have been plied have generally contained sections where the original filament bundles have less overall intra-bundle entanglement, i.e., the separately spun bundles retain some of their separate "bundle integrity". This phenomenon has been recognized. For example, when separate bundles of filaments of different polymers (homopolymer and a cationic dyeable modified polymer), dpf, and cross-sections, have been spun and then the separate bundles have been co-mingled into a single interlaced yarn, the along-end mixing has not been as "random" or unitary as if the mixed filaments had been spun from a single extrusion spinneret. This has been a defect of plied yarns, that has led to nonuniform dyed fabrics and poorer down-stream textile processing. Each separately-spun bundle of filaments does not generally entirely lose its "bundle integrity", even after such separately-spun bundles have been interlaced together and mingled into a single yarn. In contrast, the HFC yarns of the invention have shown more unitary interlace because all the filaments of the HFC yarn were spun from a single spinneret; they do not have residual "bundle integrity" from having been spun from different spinnerets. This difference between a plied yarn and a yarn of unitary interlace (all filaments spun from a single spinneret and interlaced therefrom into a single filament bundle only) is demonstrated in Example 6, hereinafter.

### EXAMPLE 2

A 255 denier 200 filament draw-feed yarn prepared by melt-spinning 21.2 LRV polyester at 288 C from a spinneret having a FED of 7.8 filaments per cm², through capillaries of LxD dimensions of 7x21 mil (0.2756 mm x 0.8268mm), the freshly-extruded filaments being protected by a short 3 cm shroud and then quenched using a radial unit having a laminar air flow rate of 22.8 m/min, the quenched filaments being converged into a unitary bundle by use of metered finish tip applicator guides and withdrawn at a spin speed of 2195 m/min, was draw false-twist textured on a Barmag FK900 using polyurethane discs (D-ring), except where indicated, at 450-500 meters per minute by process A (conventional) and by process B (modified threadline path according to one aspect of the invention). Table II summarizes process conditions; namely draw ratio; disc-to-yarn (DY) surface speed ratio was 1.707; heater temperature (Temp, in degrees centigrade); disc stack configuration (C denotes a ceramic disc was used instead of a polyurethane disc); pre/post disc tensions in grams (T1/T2) (no value was measured in some instances); and numbers of broken filaments (Frays per 1000 meters). The draw feed yarns of the invention drawn at a 1.575X draw-ratio at 180°C using a 1/7/1 disc stack (process B) gave a textured yarn having a yarn denier of 164 (0.82 dpf), a tenacity of 3.69 g/d, and elongation-to-break of 43.5%, giving a normalized (T_{B})ₙ of 5.3 g/dd, according to the invention.

### EXAMPLE 3

A 220 denier/325 filament yarn and a 220 denier/250 filament yarn were prepared (essentially as in Example 2, except that the 325 filaments were spun at a FED of 10.3 filaments per cm², and the 250 filaments at a FED of 9.74 filaments per cm²) and were draw false-twist textured on a Barmag FK900 (which has a "bent" double heater configuration) at 450-500 meters per minute at 160°C, using polyurethane discs (D-ring) with a 1.707 disc/yarn ratio (D/Y), other details being given in Table III. The quality of the textured yarns is represented by the normalized tenacity-at-break-denier (T_{B})ₙ and in the number of "Frays" per 1000 meters. The yarns were textured using the commercial threadline path (Process A) and by a modified threadline path using Process B, discussed hereinbefore. The yarns textured by Process A had (T_{B})ₙ values less than 4 g/dd and fray values significantly greater than 100, in contrast to significantly improved values from Process B (higher (T_{B})ₙ values and very low Fray Counts, less than 10).

### EXAMPLE 4

HFC as-spun yarns of filament deniers less than 1 were spun from 2G-T polyester polymer of nominal 21.2 LRV and having a zero-shear melting point Tₘ^{o} of 255 C. Process and product details are summarized in Table IV. Yarns having a DTV less than 0.75% are denoted by a letter "P" for preferred. Yarns having a preferred normalized tenacity at break denier (T_{B})ₙ of at least 6 g/dd are denoted by a letter "T". Yarns 1-5 were of 168 filaments and spun from spinnerets having a FED of 6.54/cm²; yarns 6-27 were of 200 filaments and spun from spinnerets having a FED of 7.8/cm²; yarns 28-74 were of 250 filaments and spun from spinnerets having a FED of 9.73/cm². Yarns 1, 6-17, and 28-50 were spun using 7 x 21 mil (0.178 x 0.0.533 mm) spinneret capillaries and yarns 2-5, 18-27, and 50-74 were melt-spun using 9 x 36 mil (0.229 x 0.914 mm) spinneret capillaries.

The high filament count yarns in this Example 4 have filament deniers less than 1. Many may be drawn to filament deniers of less than 0.5, and even less than 0.3 dpf. Yarns #s 3 and 5 have boil-off shrinkages of 11.4 and 4.2, respectively, and may be used, if desired, without drawing and heat setting as direct-use yarns, or the yarns may be used as draw-feed yarns, as described in U.S. Patents. Nos. 5,067,447, 5,244,616, 5,145,616, 5,223,197, and 5,250,245.

### EXAMPLE 5

Soft bulky yarns (and fabrics therefrom) are provided from use of mixed-filament yarns comprised of filaments of differing shrinkages, typically from differences in denier, and/or surface to volume ratio (i.e., cross-sectional shape), with low shrinkage fine filaments (A) providing a desirable soft surface of the bulky yarn and higher denier filaments (B) providing the fabric with improved "body" and "drape" (i.e., less "mushy"). Mixed-shrinkage high filament count yarns of the invention are illustrated for simplicity as being comprised of two filament types of differing (dpf)ₛ. On drawing the spun yarn to an elongation-to-break (E_{B}) of 25%, for example, the drawn filament deniers (dpf)_{D} are given by the expression ${\text{(dpf)}}_{\text{D}} {\text{= {(dpf)}}_{\text{s}} {\text{x [(1.25/(RDR)}}_{\text{s}} \text{]}}$; wherein the values of (dpf)_{D} for both filament types are desirably less than 1. To provide for differential shrinkage for round filaments the two filament types should differ in their spun (dpf)ₛ, with the high shrinkage filaments (B) being of higher dpf than of the low shrinkage filaments (A). To spin a single-end high filament count filament bundle of differing (dpf)ₛ, the spinneret capillary dimensions are selected to provide the desired difference, where the ratio of (dpf)ₛ is related to the ratio of spinneret dimensions according to the expression:${\text{(dpf)}}_{\text{B}} {\text{/(dpf)}}_{\text{A}} {\text{= [(L/D}}^{\text{4}} {\text{)}}_{\text{A}} {\text{/(L/D}}^{\text{4}} {\text{)}}_{\text{B}} {\text{]}}^{\text{n}} \text{,}$ where the exponent "n" equals "1" for Newtonian fluid-like behavior. This can be determined experimentally, by spinning through two capillaries of different dimensions in the same spinneret, by the expression:-${\text{n=log}}_{\text{10}} {\text{{(dpf)}}_{\text{A}} {\text{/(dpf)}}_{\text{B}} {\text{}/log}}_{\text{10}} {\text{{(L/D}}^{\text{4}} {\text{)}}_{\text{B}} {\text{/(L/D}}^{\text{4}} {\text{)}}_{\text{A}} \text{}}$ For non-round cross-sections, spun from short (shape-forming) orifice capillaries after first passing through metering capillaries, the determining value of (L/D⁴) has been that of the metering capillaries, rather than of the shape-forming capillaries. As technology advances, however, it is expected that the thickness of the shape-forming plate will be increased, perhaps to a point such that a metering capillary may not be needed. From experimentation, a "round equivalent" (L/D⁴) value may be determined for any particular combination of shape-forming odd-cross-section orifice capillary and metering capillary assembly, using a technique similar to that already described.

To avoid broken filaments, it is desirable to draw to elongation-to-break values between 15% and 40%, which can be achieved by selecting a PDR appropriate to the (RDR)ₛ of the two filament types, where $\text{PDR = is the net process draw-ratio = machine draw-ratio x overfeed (or relaxation)}$.

The above mixed-filament micro-denier HFC yarns may be air-jet textured without drawing, or a drawing step may be part of a draw-air-jet (+ optional heat relaxation) texturing process.

### EXAMPLE 6

A 225 denier, 200 filament draw-feed HFC "unitary" yarn according to the invention was prepared by melt-spinning 21.5 LRV polyester at 288°C from a single 200-capillary spinneret having a FED of 7.8 filaments per cm², through capillaries of DxL dimensions of 9 x 36 mil (0.229 mm x 0.914 mm), the freshly-extruded filaments being protected by a short 4.3 cm shroud and then quenched using a radial unit having a laminar air flow rate of 22.8 m/min, the quenched filaments being converged into a unitary bundle by use of a metered finish applicator guide, withdrawn at a speed of 2446 m/min, and the filaments interlaced using an air entanglement jet operating at 36 psig. The air jet used for interlacing the filaments was a standard "stacked" jet, as illustrated generally in Figs. XI and XII of Christini et al. U.S. Pat. No. 3,936,577, that has been in commercial use for some years.

For comparison, a 255 denier 200 filament draw-feed "plied" yarn was prepared by melt-spinning 21.7 LRV polyester at 287°C through two separate spinnerets, each having a FED of 4.4 filaments per cm², through capillaries of DxL dimensions of 12 x 50 mil (0.305 mm x 1.27 mm), the freshly extruded filaments being air quenched, and separately converged into two 100-filament bundles by use of metered finish tip applicator guides, and both withdrawn at the same speed of 2624 m/min, and the separate 100-filament bundles were then plied into a 200 filament bundle using the same type of air entanglement jet used for the HFC yarn, said jet operating at 42 psig to achieve a similar average interlace nodes/meter as for the HFC yarn. This yarn is referred to below as the "Plied" yarn.

Six HFC yarn packages and six Plied yarn packages produced as described were analyzed using a Fibrescan FS 100, supplied by Fibre Vision, Inc. to compare interlace character. 66.7 meters of each yarn package were measured at a yarn speed of 1650 m/minute, and the results are recorded in the following Table.

| | Unitary Yarns | Plied Yarns |
|---|---|---|
| Average Number of Nips per Meter | 16.6 | 17.8 |
| Average Distance Between Nips (mm) | 60.1 | 56.2 |
| Average Maximum Distance Between Nips (mm) | 228.6 | 231.7 |

As can be seen, these results seem somewhat comparable, when considering only averages measured over all 6 packages. When, however, the uniformity of the yarns is considered, by noting the maximum distance between nips and the package to package % CV of these maximum distances, the HFC yarn of the invention was shown to have significantly superior uniformity. This significant improvement in along-end uniformity also shows up in better processibility.

| | Unitary Yarns | Plied Yarns |
|---|---|---|
| Maximum Distance Between Nips (mm) | 279.3 | 314.0 |
| Package-to-Package %CV of Maximum Distance Between Nips | 12.6 | 24.0 |

**TABLE II**

| Item No. | Process Type | Temp °C | T1/T2 | Disc Stack | Draw Ration | # Frays 1000m |
|---|---|---|---|---|---|---|
| 1 | A | 160 | 30/10 | 1/7/1 | 1.409 | 10.3 |
| 2 | A | 170 | ----- | 1/71/ | 1.409 | 15.1 |
| 3 | A | 170 | 35/10 | 1/7/1 | 1.478 | 16.0 |
| 4 | A | 170 | ------ | 1/7/1 | 1.478 | 22.9 |
| 5 | A | 180 | 32/8 | 1C/7/1 | 1.478 | 9.4 |
| 6 | B | 180 | 32/8 | 1/7/1 | 1.478 | 0 |
| 7 | B | 170 | ----- | 1/7/1 | 1.478 | 0 |
| 8 | B | 180 | ----- | 1/7/1 | 1.478 | 0 |
| 9 | B | 190 | ----- | 1/7/1 | 1.478 | 0.1 |
| 10 | B | 200 | ----- | 1/7/1 | 1.478 | 0.3 |
| 11 | B | 200 | --/28 | 2/4/1 | 1.487 | 5.7 |
| 12 | B | 200 | --/12 | 2/6/1 | 1.487 | 0.4 |
| 13 | B | 200 | ------ | 1/4/1 | 1.487 | 5.7 |
| 14 | B | 200 | --/17 | 2/6/1 | 1.575 | 5.2 |
| 15 | B | 200 | --/14 | 1/7/1 | 1.575 | 2.0 |
| 16 | B | 190 | ------ | 1/7/1 | 1.575 | 1.4 |
| 17 | B | 180 | ------ | 1/7/1 | 1.575 | 0.7 |
| 18 | A | 180 | ------ | 2/6/1 | 1.575 | 200 |

**TABLE III**

| Feed yarn Properties | | | Draw Texturing Process | | | Textured Yarn Properties | | | |
|---|---|---|---|---|---|---|---|---|---|
| Yarn Count | (dpf)s | Type | T1/T2 | Disc Stack | Draw Ratio | (dpf)_{D} | Eb % | TBn g/dd | # Frays 1000 m |
| 220-325 | 0.69 | A | 52/54 | 2/5/1 | 1.409 | 0.51 | 13.9 | 1.79 | 954 |
| 220-325 | 0.69 | B | 55/54 | 1/7/1 | 1.379 | 0.51 | 38.8 | 4.22 | 1.4 |
| 220-250 | 0.88 | A | 38/20 | 2/5/1 | 1.409 | 0.66 | 29.5 | 3.23 | 474 |
| 220-250 | 0.88 | B | 50/40 | 1/7/1 | 1.379 | 0.66 | 50.8 | 5.08 | 1.4 |

## Claims

1. A process of preparing an interlaced multifilament yarn of at least 150 fine filaments in number and of 0.5 to 2.2 spun denier per filament (dpf)ₛ, from a polyester polymer of 13 to 23 relative viscosity(LRV) and of 240°C to 265°C zero-shear melting point (Tₘ^{o}) comprising :-
(i) melting the polyester polymer, heating the resulting melt to a polymer temperature (Tp) that is 25°C to 55°C above the Tₘ^{o}, and filtering the heated melt;
(ii) extruding the filtered melt through at least 150 capillaries in the face of a spinneret to form at least 150 filamentary streams at a filamentary extrusion density (FED) of at least 6 filaments/cm² and at a total melt mass flow rate W, in g/min, where ${\text{W = (dpf)}}_{\text{s}} {\text{(V}}_{\text{s}} \text{)/9000}$ times the number of filaments and Vₛ is the spinning withdrawal speed and is at least 2Km/min;
(iii) protecting the freshly-extruded filamentary streams immediately below the face of the spinneret by a delay shroud (of length L_{q} cm below said face), then cooling them by quenching air of laminar velocity (Qₐ m/min), such that the Spin Factor (SF) is 0.2 to 1, where said Spin Factor (SF) is calculated according to the expression:${\text{SF = k{(LRV)[(T}}_{\text{m}} {}^{\text{o}} {\text{+25)/(Tp)]}}^{\text{6}} {\text{[(V}}_{\text{s}} {\text{)}}^{\text{2}} {\text{/(dpf)}}_{\text{s}} {\text{][(Q}}_{\text{a}} {\text{/W)}}^{\text{0.2}} {\text{][(FED)(L}}_{\text{q}} {\text{)]}}^{\text{-0.7}} {\text{]}}}^{\text{n}}$ where "k" = 2.4x10⁺⁵ and 'n' = minus (-) 0.8;
(iv) cooling the filamentary streams to a temperature below the glass transition temperature (T_{g}), converging the resulting cooled filaments into a single multifilament bundle of at least 150 filaments at a convergence distance (L_{c}, in cm) from the face of the spinneret, and interlacing the single multifilament bundle to provide an interlaced spin-oriented yarn;
and wherein the interlaced yarn is wound to form a package at a winding speed of 2 to 5 Km/min.

2. A process according to Claim 1, wherein the polymer and process conditions are selected to provide a spin-oriented yarn that has an along-end draw tension variation (DTV,%) of less than 1%; a normalized tenacity-at-break-denier (T_{B})ₙ of at least 5 grams/drawn denier (g/dd), where ${\text{(T}}_{\text{B}} {\text{)}}_{\text{n}} {\text{= Tenacity(g/d)(RDR)}}_{\text{s}} {\text{(20.8/LRV)}}^{\text{0.75}}$, where (RDR)ₛ is the residual spun draw ratio and is defined by ${\text{(RDR)}}_{\text{s}} {\text{= [1 +(E}}_{\text{B}} \text{)/100]}$, where (E_{B}) is the percentage elongation-to-break; and an along-end denier spread (DS) of less than 2.5%.

3. A process according to Claim 1, wherein the polymer and process conditions are selected to provide a spin-oriented yarn that has an along-end draw tension variation (DTV,%) of less than 1 and between [SF + 0.2] and [SF - 0.2], SF being the spin factor, as defined; a residual draw ratio (RDR)ₛ between about 1.9 and 2.6, where (RDR)ₛ is the residual spun draw ratio and is defined by ${\text{(RDR)}}_{\text{s}} {\text{= [1+ (E}}_{\text{B}} \text{)/100]}$, where (E_{B}) is the percentage elongation-to-break; and a (1-S/Sₘ) value of greater than 0.05, where S is the boil-off shrinkage and Sₘ is the maximum shrinkage potential.

4. A process according to any of Claims 1 to 3, wherein the filament extrusion density (FED) is least 6.5 filaments per cm².

5. A process according to any of Claims 1 to 4, wherein the spin-oriented yarn is drawn by a draw ratio such as to provide a drawn yarn of elongation to-break (E_{B}) 15 to 40%, and of drawn filament denier about 1 or less.

6. A process according to Claim 5, wherein a plurality of such spin-oriented yarns are drawn in the form of a weftless warp sheet.

7. A process according to Claim 5, wherein the drawing of the spin-oriented yarn is coupled with the melt-spinning, whereby the resulting drawn yarn is wound to form a package at a winding speed of 3 to 5 Km/min.

8. A process according to any of the preceding claims, wherein the polymer and process conditions are selected to provide a yarn that has a (1-S/Sₘ)-value greater than 0.85, where S is the boil-off shrinkage and Sₘ is the maximum shrinkage potential.

9. A process according to any of the preceding claims, wherein the spin-oriented yarn is draw-textured by a draw ratio such as to provide a bulky yarn of tenacity-at-break-denier (T_{B})ₙ of at least 4 g/dd, where ${\text{(T}}_{\text{B}} {\text{)}}_{\text{n}} {\text{= Tenacity(g/d)(RDR)}}_{\text{s}} {\text{(20.8/LRV)}}^{\text{0.75}}$, where (RDR)ₛ is the residual spun draw ratio and is defined by ${\text{(RDR)}}_{\text{s}} {\text{= [1 +(E}}_{\text{B}} \text{)/100]}$, where (E_{B}) is the percentage elongation-to-break; an elongation-to-break (E_{B}) of 20 to 45%; and a Fray Count of less than 10 frays per 1000 meters.

10. A process according to Claim 9, wherein a low-friction device is provided to reduce twist-induced draw in the draw-texturing threadline between the first upstream contact point and the first friction twist insertion point such as to provide a "break angle" of less than 15 degrees and to increase radius of curvature of the upstream contact to greater than 2.5 mm.

11. A process according to any of the preceding claims, wherein filaments of different deniers or cross-sections are co-spun from the same extrusion spinneret.

12. A multi-filament polyester yarn, wherein the polyester polymer has a relative viscosity (LRV) of 13 to 23 and a zero-shear melting point (Tₘ^{o}) of 240° to 265°C; comprising at least 150 flat filaments of denier 0.5 to 2.2, and having an elongation-to-break (E_{B}) of 40 to 160%, and a normalized yarn tenacity-at-break-denier (T_{B})ₙ of at least 5 g/dd, where ${\text{(T}}_{\text{B}} {\text{)}}_{\text{n}} {\text{= Tenacity(g/d)(RDR)}}_{\text{s}} {\text{(20.8/LRV)}}^{\text{0.75}}$, and where (RDR)ₛ is the residual spun draw ratio and is defined by ${\text{(RDR)}}_{\text{s}} {\text{=[1+(E}}_{\text{B}} \text{)/100]}$, characterised in that the filament entanglement of said yarn shows unitary interlace, and the yarn has an along-end draw tension coefficient of variation (DTV,%) of less than 1%.

13. A yarn according to Claim 12, having an elongation-to-break (E_{B}) of 40 to 90%, and a (1-S/Sₘ) value of at least 0.85, where S is the boil-off shrinkage and Sₘ is the maximum shrinkage potential.

14. A multi-filament polyester yarn, wherein the polyester polymer has a relative viscosity (LRV) of 13 to 23 and a zero-shear melting point (Tₘ^{o}) of 240° to 265°C; comprising at least 150 flat filaments of denier 0.2 to 1, and having an elongation-to-break (E_{B}) of 15 to 40%, and a normalized yarn tenacity-at-break-denier (T_{B})ₙ of at least 5 g/dd, where ${\text{(T}}_{\text{B}} {\text{)}}_{\text{n}} {\text{= Tenacity(g/d)(RDR)}}_{\text{s}} {\text{(20.8/LRV)}}^{\text{0.75}}$, and where (RDR)ₛ is the residual spun draw ratio and is defined by ${\text{(RDR)}}_{\text{s}} {\text{= [1 +(E}}_{\text{B}} \text{)/100]}$, characterised in that the filament entanglement of said yarn shows unitary interlace, and the yarn has an along-end draw tension coefficient of variation (DTV,%) of less than 1 %.

15. A multi-filament polyester yarn, wherein the polyester has a relative viscosity (LRV) of 13 to 23 and a zero-shear melting point (Tₘ^{o}) of 240° to 265°C; comprising at least 150 textured filaments of denier 0.2 to 1, and having an elongation-to-break (E_{B}) of 15% to 45%, and a normalized tenacity-at-break-denier (T_{B})ₙ of at least 4 g/dd, where ${\text{(T}}_{\text{B}} {\text{)}}_{\text{n}} {\text{= Tenacity(g/d)(RDR)}}_{\text{s}} {\text{(20.8/LRV)}}^{\text{0.75}}$, and where (RDR)ₛ is the residual spun draw ratio and is defined by ${\text{(RDR)}}_{\text{s}} {\text{= [1 +(E}}_{\text{B}} \text{)/100]}$, characterised in that the filament entanglement of said yarn shows unitary interlace, and the yarn has a Fray Count of less than 10 per 1000 meters.

## Patentansprüche

1. Verfahren zur Herstellung eines verflochtenen Multifilgarnes mit einer Anzahl von mindestens 150 feinen Elementarfäden und mit 0,5 bis 2,2 ersponnenem Denier pro Elementarfaden (dpf)ₛ aus einem Polyesterpolymer mit einer relativen Viskosität (LRV) von 13 bis 23 und einem Schmelzpunkt (Tₘ^{o}) bei Nullscherung von 240°C bis 265°C, das aufweist:
(i) Schmelzen des Polyesterpolymers, Erwärmen der resultierenden Schmelze auf eine Polymertemperatur (Tp), die 25°C bis 55°C über der Tₘ^{o} liegt, und Filtrieren der erwärmten Schmelze;
(ii) Extrudieren der filtrierten Schmelze durch mindestens 150 Kapillaren in der Oberfläche einer Spinndüse, um mindestens 150 Elementarfadenströme mit einer Elementarfadenextrudierdichte (FED) von mindestens 6 Elementarfäden/cm² und einer Strömungsmenge W der gesamten Schmelzmasse in g/min. zu bilden, worin sind: ${\text{W = (dpf)}}_{\text{s}} \text{(Vs)/9000}$ mal der Anzahl der Elementarfäden und Vₛ die Spinnabsauggeschwindigkeit, und sie beträgt mindestens 2 km/min.;
(iii) Schützen der frisch extrudierten Elementarfadenströme unmittelbar unterhalb der Oberfläche der Spinndüse durch eine Verzögerungsabdeckung (mit der Länge L_{q} cm unterhalb der Oberfläche), danach Abkühlen dieser durch Abschreckluft mit einer laminaren Geschwindigkeit (Qₐ m/min.), so daß der Spinnfaktor (SF) 0,2 bis 1 beträgt, wobei der Spinnfaktor (SF) gemäß dem folgenden Ausdruck berechnet wird:${\text{SF = k{(LRV)[(T}}_{\text{m}} {}^{\text{o}} {\text{+25)/(T}}_{\text{P}} {\text{)]}}^{\text{6}} {\text{[(V}}_{\text{s}} {\text{)}}^{\text{2}} {\text{/(dpf)}}_{\text{s}} {\text{)][(Q}}_{\text{a}} {\text{/W)}}^{\text{0.2}} {\text{][(FED)(L}}_{\text{q}} {\text{)]}}^{\text{-0.7}} {\text{]}}}^{\text{n}}$ worin sind: "k" = 2,4 x 10⁺⁵ und 'n' = minus (-) 0,8;
(iv) Abkühlen der Elementarfadenströme auf eine Temperatur unterhalb der Glasumwandlungstemperatur (T_{g}), Konvergieren der resultierenden abgekühlten Elementarfäden zu einem einzelnen Multifilbündel von mindestens 150 Elementarfäden bei einem Konvergenzabstand (L_{c}, in cm) von der Oberfläche der Spinndüse, und Verflechten des einzelnen Multifilbündels, um ein verflochtenes spinnorientiertes Garn zu liefern;
und worin das verflochtene Garn mit einer Aufwickelgeschwindigkeit von 2 bis 5 km/min. aufgewickelt wird, um einen Wickelkörper zu bilden.

2. Verfahren nach Anspruch 1, bei dem das Polymer und die Verfahrensbedingungen so ausgewählt werden, daß ein spinnorientiertes Garn geliefert wird, das aufweist: eine Reckspannungsabweichung (DTV,%) längs des Fadens von weniger als 1%; einen normalisierten Bruchfestigkeitsdenier (T_{B})ₙ von mindestens 5 Gramm/gerecktem Denier (g/dd), worin ist ${\text{(T}}_{\text{B}} {\text{)}}_{\text{n}} {\text{= Festigkeit (g/d)(RDR)}}_{\text{s}} {\text{(20,8/LRV)}}^{\text{0,75}}$, worin (RDR)ₛ das Restspinnreckverhältnis ist und definiert wird durch ${\text{(RDR)}}_{\text{s}} {\text{= [1+(E}}_{\text{B}} \text{)/100]}$, worin (E_{B}) die prozentuale Bruchdehnung ist; und eine Denierstreuung (DS) längs des Fadens von weniger als 2,5%.

3. Verfahren nach Anspruch 1, bei dem das Polymer und die Verfahrensbedingungen so ausgewählt werden, daß ein spinnorientiertes Garn geliefert wird, das aufweist: eine Reckspannungsabweichung (DTV,%) längs des Fadens von weniger als 1 und zwischen [SF+0,2] und [SF-0,2], wobei SF der Spinnfaktor ist, wie er definiert wird; ein Restreckverhältnis (RDR)ₛ zwischen etwa 1,9 und 2,6, worin (RDR)ₛ das Restspinnreckverhältnis ist und definiert wird durch ${\text{(RDR)}}_{\text{s}} {\text{= [1+(E}}_{\text{B}} \text{)/100]}$, worin (E_{B}) die prozentuale Bruchdehnung ist; und einen (1-S/Sₘ)-Wert von mehr als 0,05, worin S die Abkochschrumpfung und Sₘ das maximale Schrumpfungspotential sind.

4. Verfahren nach einem der Ansprüche 1 bis 3, bei dem die Elementarfadenextrudierdichte (FED) mindestens 6,5 Elementarfäden pro cm² beträgt.

5. Verfahren nach einem der Ansprüche 1 bis 4, bei dem das spinnorientierte Garn mittels eines Reckverhältnisses so gereckt wird, daß ein gerecktes Garn mit einer Bruchdehnung (E_{B}) von 15 bis 40% und mit einem gereckten Elementarfadendenier von etwa 1 oder Meiner bereitgestellt wird.

6. Verfahren nach Anspruch 5, bei dem eine Vielzahl derartiger spinnorientierter Garne in der Form eines schußlosen Kettfadenflächengebildes gereckt wird.

7. Verfahren nach Anspruch 5, bei dem das Recken des spinnorientierten Garnes mit dem Schmelzspinnen verbunden ist, wobei das resultierende gereckte Garn mit einer Aufwickelgeschwindigkeit von 3 bis 5 km/min. aufgewickelt wird, um einen Wickelkörper zu bilden.

8. Verfahren nach einem der vorhergehenden Ansprüche, bei dem das Polymer und die Verfahrensbedingungen so ausgewählt werden, daß ein Garn bereitgestellt wird, das einen (1-S/Sₘ)-Wert von mehr als 0,85 aufweist, worin S die Abkochschrumpfung und Sₘ das maximale Schrumpfungspotential sind.

9. Verfahren nach einem der vorhergehenden Ansprüche, bei dem das spinnorientierte Garn mit einem Reckverhältnis so recktexturiert wird, daß ein bauschiges Garn geliefert wird mit: einem Bruchfestigkeitsdenier (T_{B})ₙ von mindestens 4 g/dd, worin ${\text{(T}}_{\text{B}} {\text{)}}_{\text{n}} {\text{= Festigkeit (g/d)(RDR)}}_{\text{s}} {\text{(20,8/LRV)}}^{\text{0,75}}$, worin (RDR)ₛ das Restspinnreckverhältnis ist und durch ${\text{(RDR)}}_{\text{s}} {\text{= [1+(E}}_{\text{B}} \text{)/100]}$ definiert wird, worin (E_{B}) die prozentuale Bruchdehnung ist; einer Bruchdehnung (E_{B}) von 20 bis 45%; und einer Ausfransungszahl von weniger als 10 Ausfransungen pro 1000 Meter.

10. Verfahren nach Anspruch 9, bei dem eine Vorrichtung mit geringer Reibung bereitgestellt wird, um das durch die Drehung herbeigeführte Recken im Recktexturierfadenverlauf zwischen der ersten stromaufwärts gelegenen Kontaktstelle und der ersten Reibungsdrehungseinbringungsstelle so zu verringern, daß ein "Bruchwinkel" von weniger als 15 Grad bewirkt und der Krümmungsradius des stromaufwärts gelegenen Kontaktes aufmehr als 2,5 mm vergrößert wird.

11. Verfahren nach einem der vorhergehenden Ansprüche, bei dem Elementarfäden mit unterschiedlichem Denier oder unterschiedlichen Querschnitten gemeinsam aus der gleichen Extrudierspinndüse ersponnen werden.

12. Multifilpolyestergarn, bei dem das Polyesterpolymer eine relative Viskosität (LRV) von 13 bis 23 und einen Schmelzpunkt (Tₘ^{o}) bei Nullscherung von 240 bis 265°C aufweist; das mindestens 150 flache Elementarfäden aufweist, die einen Denier von 0,5 bis 2,2 und eine Bruchdehnung (E_{B}) von 40 bis 160% sowie einen normalisierten Garnbruchfestigkeitsdenier (T_{B})ₙ von mindestens 5 g/dd zeigen, worin ${\text{(T}}_{\text{B}} {\text{)}}_{\text{n}} {\text{= Festigkeit (g/d)(RDR)}}_{\text{s}} {\text{(20,8/LRV)}}^{\text{0,75}}$, worin (RDR)ₛ das Restspinnreckverhältnis ist und durch ${\text{(RDR)}}_{\text{s}} {\text{= [1+(E}}_{\text{B}} \text{)/100]}$ definiert wird, dadurch gekennzeichnet, daß die Elementarfadenverhakung des Garnes eine unitäre Verflechtung zeigt, und das Garn einen Reckspannungsvariationskoeffizienten (DTV,%) längs des Fadens von weniger als 1% aufweist.

13. Garn nach Anspruch 12, das eine Bruchdehnung (E_{B}) von 40 bis 90% und einen (1-S/Sₘ)-Wert von mindestens 0,85 zeigt, worin S die Abkochschrumpfung und Sₘ das maximale Schrumpfungspotential sind.

14. Multifilpolyestergarn, bei dem das Polyesterpolymer eine relative Viskosität (LRV) von 13 bis 23 und einen Schmelzpunkt (Tₘ^{o}) bei Nullscherung von 240 bis 265°C aufweist; das mindestens 150 flache Elementarfäden aufweist, die einen Denier von 0,2 bis 1 und eine Bruchdehnung (E_{B}) von 15 bis 40% sowie einen normalisierten Garnbruchfestigkeitsdenier (T_{B})ₙ von mindestens 5 g/dd zeigen, worin ${\text{(T}}_{\text{B}} {\text{)}}_{\text{n}} {\text{= Festigkeit (g/d)(RDR)}}_{\text{s}} {\text{(20,8/LRV)}}^{\text{0,75}}$, worin (RDR)ₛ das Restspinnreckverhältnis ist und durch ${\text{(RDR)}}_{\text{s}} {\text{= [1+(E}}_{\text{B}} \text{)/100]}$ definiert wird, dadurch gekennzeichnet, daß die Elementarfadenverhakung des Garnes eine unitäre Verflechtung zeigt, und das Garn einen Reckspannungsvariationskoeffizienten (DTV, %) längs des Fadens von weniger als 1% aufweist.

15. Multifilpolyestergarn, bei dem das Polyester eine relative Viskosität (LRV) von 13 bis 23 und einen Schmelzpunkt (Tₘ^{o}) bei Nullscherung von 240 bis 265°C aufweist; das mindestens 150 texturierte Elementarfäden aufweist, die einen Denier von 0,2 bis 1 und eine Bruchdehnung (E_{B}) von 15 bis 45% sowie einen normalisierten Bruchfestigkeitsdenier (T_{B})ₙ von mindestens 4 g/dd zeigen, worin ${\text{(T}}_{\text{B}} {\text{)}}_{\text{n}} {\text{= Festigkeit (g/d)(RDR)}}_{\text{s}} {\text{(20,8/LRV)}}^{\text{0,75}}$, worin (RDR)ₛ das Restspinnreckverhältnis ist und durch ${\text{(RDR)}}_{\text{s}} {\text{= [1+(E}}_{\text{B}} \text{)/100]}$ definiert wird, dadurch gekennzeichnet, daß die Elementarfadenverhakung des Garnes eine unitäre Verflechtung zeigt, und das Garn eine Ausfransungszahl von weniger als 10 pro 1000 Meter aufweist.

## Revendications

1. Procédé de préparation d'un fil multifilament entrelacé contenant un nombre d'au moins 150 filaments fins et ayant un denier filé par filament (dpf)ₛ compris entre 0,5 et 2,2, à partir d'un polymère de polyester d'une viscosité relative (LRV) comprise entre 13 et 23 et avec un point de fusion sans cisaillement (Tₘ^{o}) compris entre 240°C et 265°C, comprenant les étapes ci-dessous:
(i) fusion du polymère de polyester, chauffage du polymère fondu résultant à une température de polymère (Tp) dépassant de 25°C à 55°C le Tₘ^{o} et filtration du polymère fondu chauffé;
(ii) extrusion du polymère fondu filtré à travers au moins 150 capillaires dans la face d'une filière pour former au moins 150 courants de filaments, avec une densité d'extrusion des filaments (FED)) d'au moins 6 filaments/cm² et un débit massique total W du polymère fondu, en g/minute, ${\text{W = (dpf)}}_{\text{S}} {\text{(V}}_{\text{S}} \text{)/9000}$ fois le nombre des filaments et V_{S} représentant la vitesse de prélèvement de filage et correspondant à au moins 2 km/minute;
(iii) protection des courants de filaments venant d'être extrudés immédiatement au-dessous de la face de la filière par une enveloppe de ralentissement (d'une longueur de L_{q} cm au-dessous de ladite face), avant leur refroidissement par de l'air de trempe d'une vitesse laminaire de (Qₐ m/minute), de sorte que le facteur de filage (SF) est compris entre 0,2 et 1, ledit facteur de filage (SF) étant calculé selon l'expression:${\text{SF = k{(LRV)[T}}_{\text{m}} {}^{\text{o}} {\text{+25)/(Tp)]}}^{\text{6}} {\text{[(V}}_{\text{S}} {\text{)}}^{\text{2}} {\text{/(dpf)}}_{\text{S}} {\text{][(Q}}_{\text{a}} {\text{/W)}}^{\text{0,2}} {\text{][(FED)(L}}_{\text{q}} {\text{)]}}^{\text{0,7}} {\text{]}}}^{\text{n}}$ où "k" = 2,4x10⁺⁵ et 'n' = moins (-) 0,8;
(iv) refroidissement des courants de filaments à une température inférieure à la température de transition vitreuse (T_{g}), rassemblement des filaments refroidis résultants en un seul faisceau multifilaments contenant au moins 150 filaments à une distance de convergence (L_{c} en cm) de la face de la filière, et entrelacement du seul faisceau multifilaments pour produire un fil entrelacé à orientation de filage;
le fil entrelacé étant enroulé pour former un enroulement à une vitesse d'enroulement comprise entre 2 et 5 km/minute.

2. Procédé selon la revendication 1, dans lequel le polymère et les conditions de traitement sont sélectionnés de sorte à fournir un fil à orientation de filage ayant une variation de la tension d'étirage le long des fils (DTV, %) inférieure à 1%; un denier de la ténacité à la rupture normalisé (T_{B})ₙ d'au moins 5 grammes/denier étiré (g/dd), ${\text{(T}}_{\text{B}} {\text{)}}_{\text{n}} {\text{= ténacité(g/d)(RDR)}}_{\text{s}} {\text{(20,8/LRV)}}^{\text{0,75}}$, (RDR)ₛ représentant le taux d'étirage de filage résiduel et étant défini par ${\text{(RDR)}}_{\text{s}} {\text{= [1+E}}_{\text{B}} \text{)/100]}$, (E_{B}) représentant le pourcentage de l'allongement à la rupture; et une distribution du denier le long des fils (DS) inférieure à 2,5%.

3. Procédé selon la revendication 1, dans lequel le polymère et les conditions de traitement sont sélectionnés de sorte à fournir un fil à orientation de filage ayant une variation de la tension d'étirage le long des fils (DTV, %) inférieure à 1 et comprise entre [SF + 0,2] et [SF - 0,2], SF représentant le facteur de filage, comme défini; un taux d'étirage résiduel (RDR)ₛ compris entre environ 1,0 et 2,6, (RDR)ₛ représentant le taux d'étirage de filage résiduel et étant défini par ${\text{(RDR)}}_{\text{s}} {\text{= [1+(E}}_{\text{B}} \text{)/100],}$ (E_{B}) représentant le pourcentage de l'allongement à la rupture; et une valeur (1-S/Sₘ) supérieure à 0,05, S représentant le retrait par évaporation et Sₘ représentant le potentiel de retrait maximal.

4. Procédé selon l'une quelconque des revendications 1 à 3, dans lequel la densité d'extrusion des filaments (FED) représente au moins 6,5 filaments par cm².

5. Procédé selon l'une quelconque des revendications 1 à 4, dans lequel le fil à orientation de filage est étiré à un taux d'étirage tel à produire un fil étiré ayant un allongement à la rupture (E_{B}) compris entre 15 et 40% et un denier du filament étiré de l'ordre de 1 ou moins.

6. Procédé selon la revendication 5, dans lequel plusieurs de ces fils à orientation de filage sont étirés sous forme d'une feuille de chaîne sans trame.

7. Procédé selon la revendication 5, dans lequel l'étirage du fil à orientation de filage est couplé avec le filage par fusion, le fil étiré résultant étant ainsi enroulé pour former un enroulement à une vitesse d'enroulement comprise entre 3 à 5 km/minute.

8. Procédé selon l'une quelconque des revendications précédentes, dans lequel le polymère et les conditions de traitement sont sélectionnés de sorte à produire un fil ayant une valeur (1-S/Sₘ) supérieure à 0,85, S représentant le retrait par évaporation et Sₘ représentant le potentiel de retrait maximal.

9. Procédé selon l'une quelconque des revendications précédentes, dans lequel le fil à orientation de filage est texturé par étirage à un taux d'étirage tel à produire un fil gonflant ayant un denier de la ténacité à la rupture (T_{B})ₙ d'au moins 4 g/dd, (${\text{T}}_{\text{B}} {\text{)}}_{\text{n}} {\text{= ténacité (g/d)(RDR)}}_{\text{s}} {\text{(20,8/LRV)}}^{\text{0,75}}$, (RDR)ₛ représentant le taux d'étirage de filage résiduel et étant défini par ${\text{(RDR)}}_{\text{s}} {\text{= [1+ (E}}_{\text{B}} \text{)/100]}$, (E_{B}) représentant le pourcentage de l'allongement à la rupture; un allongement à la rupture (E_{B}) compris entre 20 et 45%, et un nombre d"éraillures (Fray Count) de moins de 10 éraillures par 1000 mètres.

10. Procédé selon la revendication 9, dans lequel un dispositif à frottement réduit est fourni pour réduire l'étirage entraîné par la torsion dans le parcours du fil lors de la texturation par étirage entre le premier point de contact en amont et le premier point d'insertion de torsion à frottement, de sorte à établir un "angle de moindre cassure" de moins de 15% et à accroître le rayon de courbure du contact en amont à plus de 2,5 mm.

11. Procédé selon l'une quelconque des revendications précédentes, dans lequel des filaments ayant des deniers différents et des sections transversales différentes sont filés ensemble à partir de la même filière d'extrusion.

12. Fil multifilament en polyester, dans lequel le polymère de polyester a une viscosité relative (LRV) comprise entre 13 et 23 et un point de fusion sans cisaillement (Tₘ^{o}) compris entre 240° et 265°C; comprenant au moins 150 filaments plats d'un denier compris entre 0,5 et 2,2; et ayant un allongement à la rupture (E_{B}) compris entre 40 et 160%, et un denier de la ténacité à la rupture de fil normalisé (T_{B})ₙ d'au moins 5 g/dd, ${\text{(T}}_{\text{B}} {\text{)}}_{\text{n}} {\text{= ténacité (g/d) (RDR)}}_{\text{s}} {\text{(20,8/LRV)}}^{\text{0,75}}$, (RDR)ₛ représentant le taux d'étirage de filage résiduel et étant défini par ${\text{(RDR)}}_{\text{s}} {\text{= [1+ (E}}_{\text{B}} \text{)/100]}$, caractérisé en ce que l'enchevêtrement des filaments dudit fil présente un entrelacement unitaire, le fil ayant un coefficient de variation de la tension d'étirage le long des fils (DTV, %) inférieur à 1%.

13. Fil selon la revendication 12, ayant un allongement à la rupture (E_{B}) compris entre 40 et 90%, et une valeur (1-S/Sₘ) d'au moins 0,85, S représentant le retrait par évaporation et Sₘ représentant le pourcentage de retrait maximal.

14. Fil multifilament en polyester, dans lequel le polymère de polyester a une viscosité relative (LRV) comprise entre 13 et 23 et un point de fusion sans cisaillement (Tₘ^{o}) compris entre 240° et 265°C; comprenant au moins 150 filaments plats d'un denier compris entre 0,2 et 1; et ayant un allongement à la rupture (E_{B}) compris entre 15 et 40%, et un denier de la ténacité à la rupture de fil normalisé (T_{B})ₙ d'au moins 5 g/dd, ${\text{(T}}_{\text{B}} {\text{)}}_{\text{n}} {\text{= ténacité (g/d) (RDR)}}_{\text{s}} {\text{(20,8/LRV)}}^{\text{0,75}}$, (RDR)ₛ représentant le taux d'étirage de filage résiduel et étant défini par ${\text{(RDR)}}_{\text{s}} {\text{= [1+ (E}}_{\text{B}} \text{)/100]}$, caractérisé en ce que l'enchevêtrement des filaments dudit fil présente un entrelacement unitaire, le fil ayant un coefficient de variation de la tension d'étirage le long des fils (DTV, %) inférieur à 1%.

15. Fil multifilament en polyester, dans lequel le polyester a une viscosité relative (LRV) comprise entre 13 et 23 et un point de fusion sans cisaillement (Tₘ^{o}) compris entre 240° et 265°C; comprenant au moins 150 filaments texturés d'un denier compris entre 0,2 et 1; et ayant un allongement à la rupture (E_{B}) compris entre 15% et 45%, et un denier de la ténacité à la rupture normalisé (T_{B})ₙ d'au moins 4 g/dd, ${\text{(T}}_{\text{B}} {\text{)}}_{\text{n}} {\text{= ténacité (g/d) (RDR)}}_{\text{s}} {\text{(20,8/LRV)}}^{\text{0,75}}$, (RDR)ₛ représentant le taux d'étirage de filage résiduel et étant défini par ${\text{(RDR)}}_{\text{s}} {\text{= [1+ (E}}_{\text{B}} \text{)/100}$, caractérisé en ce que l'enchevêtrement des filaments dudit fil présente un entrelacement unitaire, le fil ayant un nombre d'éraillures inférieur à 10 par 1000 mètres.
